

## UNITED STATES PATENT OFFICE

2,507,475

## ELECTRODEPOSITION OF CHROMIUM

Rex R. Lloyd, Boulder City, Nev., assignor, by  
mesne assignments, to Crimora Research & De-  
velopment Corporation, New York, N. Y., a cor-  
poration of Virginia.

No Drawing. Application February 4, 1946,  
Serial No. 645,473

1 Claim. (CL 204—105)

1

The present invention relates to the electrodeposition of chromium and, more particularly, to the electrowinning of chromium from chromium salt solutions. This application is a continuation in part of applications Ser. Nos. 578,549 and 578,551, filed February 17, 1945, now abandoned.

Heretofore, it has not been possible to recover chromium economically from chromium salt baths by electrolytic methods. For example, the use of prior methods generally has resulted in thin, usually oxide contaminated deposits at low current efficiency.

In accordance with the present invention, it is possible to plate out thick deposits of chromium of good quality which can be readily stripped from the cathode.

The present invention also makes it possible to deposit chromium uniformly and satisfactorily at a high current efficiency.

An important aim of the invention is to provide a method of electrowinning chromium which may be carried out continuously over long periods of time without materially decreasing the quality of the deposit, while maintaining a high current efficiency.

Other aims and advantages of the invention will be apparent from the following description of the invention and the appended claim.

In general, the present invention is applicable to the electrowinning of chromium from a solution containing ammonium, sodium, sulfate, chromous and chromic ions. The invention resides in the discovery that the new and improved results referred to above may be obtained by controlling the conditions of electrolysis within the ranges or limits defined more particularly hereinafter. Such conditions include, for example, the composition, purity, temperature and pH of the bath, and the current density used.

In the practice of the present invention, it is preferred, but not essential, to use an electrolytic cell divided into catholyte and anolyte compartments by means of an ion-permeable diaphragm, which type of apparatus is well known in the art. With respect to the electrodes, it is preferred to use lead or lead-alloy anodes while the cathodes preferably are of bronze containing about 88% copper and the balance tin. The particular composition of the electrodes is not critical. With respect to the anodes, for instance, it is essential only that they will not contaminate the bath during electrolysis. With respect to the cathodes, there is less danger of contamination and a wide variety of materials or combina-

2

tion of materials may be used such as graphite, lead, copper, nickel, brass, aluminum, tin and various stainless steels.

In accordance with the invention the electrolyte contains the following elements in an amount within the ranges shown:

|          | Grams per liter |
|----------|-----------------|
| Sodium   | 20 to 40        |
| Ammonium | 30 to 50        |
| Chromium | 18 to 60        |

Sulfate ion is also present in an amount at least stoichiometrically equivalent to the ammonia, sodium and chromium.

It has also been found that when the amount of chromium present exceeds about 30 grams per liter, the concentration of the sodium must be less than that of the chromium in order to obtain satisfactory results.

As a typical example of an electrolyte prepared in accordance with the invention, which is given merely by way of illustration, satisfactory results have been obtained by utilizing an electrolyte containing approximately 32 grams of chromium per liter, with sulfate ion present in the necessary stoichiometric amount.

The method of forming the electrolyte is not critical except in so far as it is necessary that the solution be substantially free of lead, aluminum and magnesium. The aqueous solution can be made conveniently, for example, by dissolving the necessary amounts of sodium sulfate, ammonium sulfate and chromium sulfate. In general, it is preferred to use chromium ammonium alum, which is readily available in pure form; although it has been found that potassium alum may be substituted for or used in combination with the ammonium alum. The preparation of this alum in a form suitable for use in the present invention, is disclosed in my copending application Ser. No. 645,474, filed February 4, 1946. The solution is stabilized in the green modification by heating for a short period at a temperature above 70° C.; but not substantially above the boiling point at atmospheric pressure.

Substitution of some of the sulfates in the electrolyte may be made with chlorides; provided enough sulfate is present to form a complex of the alum type.

At the beginning of electrolysis the chromium present will be substantially all in the trivalent state (Cr<sup>+++</sup>). As electrolysis proceeds, however, divalent chromium (Cr<sup>++</sup>) is formed. In general, the chromous ion will not accumulate to an extent beyond about 20 grams per liter, when

the total chromium is about 35 grams per liter. Satisfactory results are obtained when the chromous ion has been formed by electrolysis to a substantial extent of say, about 45% of the total chromium present. If desired, the formation of chromous ion may be expedited by omitting the ammonium sulfate from the bath during the initial period of electrolysis. Sufficient chromium should be present, however, so that the amount of chromous ion will not exceed 95% of the total chromium.

It has been found that the pH of the electrolyte is another determining factor in the successful carrying out of the present invention. It is preferred to adjust the pH of the bath to within the range of about 1.8 to 2.2. This may be accomplished without the addition of any new radicals, for example, by the addition of sulfuric acid. In general, for satisfactory results, the pH of the electrolyte should be within the range of 1.0-2.8.

The temperature of the bath is also a very important factor in accomplishing the aims of the present invention. At temperatures below 27° C., if maintained for any substantial period of time, there is a tendency to form insoluble, violet chromium salts. At temperatures above about 45° C., there is a decrease in current efficiency and the nature of the plate is also adversely affected.

The current density utilized in the cell also has a controlling influence upon the successful operation of the method of the present invention. In general, a cathodic current density in the range of about 30 to 160 amperes per square foot is necessary to obtain a good plate. If the pH is from 2.3 to 2.8, the preferred current density is 30 to 60 amperes per square foot; from pH 2.3 to 1.8, current density 50. to 100 amperes per square foot; and from pH 1.0 to 1.8, current density 100. to 160 amperes per square foot.

During the operation of the cell, it has been found, in accordance with the present invention, that a substantial increase in current efficiency and a greatly improved structure of the deposit is obtained by adding a reduced sulfur compound such as sulfur dioxide, or water-soluble sulfites, hyposulfites, sulfamites, xanthates, thionates, thiosulfates, sulfides and other sulphur compounds in which the sulfur has a valence of less than 6. The amount required to effect such improvement is very small and preferably about  $12 \times 10^{-5}$  mols per liter of any of these compounds.

An excess of reduced sulfur compounds is to be avoided. Since the reduced sulfur compounds are destroyed during electrolysis, it is necessary to replenish the amount of these compounds in the catholyte. This is preferably done continuously by adding, for example, 0.00002-0.0002 mols per liter, per hour of sulfite ion to the catholyte. Even when added in a small amount, it has been found that after several hours of cyclic operation, the accumulation of sulfur compounds has an adverse effect on the current efficiency and structure of the deposit. It is an advantage of the present invention, however, that such excess may be effectively removed without adversely affecting the electrolyte. In accordance with the invention, this is accomplished periodically by heating the electrolyte with ammonium persulfate or hydrogen peroxide at a convenient point in the circuit, outside the cell. The amount of addition agent

required is small. For example, with the preferred addition agent ammonium persulfate, only about 2 grams per liter is required to remove excess reduced sulfur compound. After such treatment, the electrolyte is suitable for re-use in the cell without further treatment.

It will be apparent that the present invention may be practiced, if desired, in the usual batch type of operation. For example, in plating, the bath could be used with an insoluble anode to plate out Cr within the concentration range 18-60 grams per liter. A soluble chromium anode could also be used to maintain the chromium concentration. However, it is preferred, and an advantage of the invention, to operate the process continuously. This may be accomplished by continuously or intermittently replacing part or all of the spent electrolyte with fresh or replenished electrolyte prepared as set forth above, or by replacing the chromium, which was removed by electroplating, in the electrolyte, for example, in accordance with the processes set forth in my copending applications Ser. No. 645,474, filed February 4, 1946, and Ser. No. 578,549, filed February 17, 1945, the latter now abandoned.

The following specific examples are given of the carrying out of the present invention, merely by way of illustration, to assist in the understanding of the invention and are not to be construed as limiting the scope of the invention:

As an example of the practice of the invention, reference is made to a test involving five weeks of continuous electrolysis using one cathode at a time. Each cathode remained in the cell 48 hours. The original electrolyte contained about 36 grams of chromium per liter, 33 grams of sodium per liter and 42 grams of ammonium per liter. It was heated to about 30° C. for about thirty minutes and cooled. The solution was circulated through the cathode compartment of a cell and the chromium was replenished to maintain the chromium content about 35 grams per liter. About 0.01 of a gram of ammonium sulphite per liter was added per hour. The average pH of the catholyte was 1.85 and the anolyte contained about 250 grams of sulphuric acid per liter. After a few hours of operation, the ratio of chromous to chromic ions was about 1 to 1. The solution contained not more than 50 milligrams per liter of magnesium and aluminum and substantially no other impurities. The average catholyte temperature was 29.5° C. and its density was about 1.26. The current density was maintained at about 70 amperes per square foot. On the average, three pounds of dense and satisfactory chromium was obtained each 24 hours at a greatly increased current efficiency with an expenditure of about 8 kilowatt hours per pound of metal. This deposited chromium was readily stripped from the cathode plate by hammering and passing a thin steel blade under the deposit.

In a similar run, in which no ammonium sulphite was added, the deposits were hard and bright. They peeled readily from the cathode, thus causing some difficulty by premature separation. Then, 0.3 to 0.4 of a gram of ammonium sulphite was added to 30 liters of catholyte. The current efficiency was increased by the hourly addition of this amount of ammonium sulphite and was maintained substantially constant. No difficulty was experienced from premature peel-

ing, and the current efficiency increased substantially.

It will be appreciated that the invention will be susceptible of many variations and modifications by one skilled in the art without departing from the spirit of the invention, and all such variations and modifications are intended to be included within the scope of the following claim.

What is claimed is:

A method of electrowinning chromium in a compartment cell comprising forming an electrolyte having a pH range of 1.8 to 2.3 and consisting of 18-60 grams of chromium per liter, 30-50 grams of ammonium per liter, 20-40 grams of sodium per liter, the amount of said sodium not exceeding the amount of said chromium when more than 30 grams of chromium per liter are present, and sulfate ion in an amount at least the stoichiometric equivalent of the chromium, sodium and ammonium, heating the electrolyte to a temperature of approximately 80° C. to stabilize the chromium sulfate in the green modification, and electrolyzing said electrolyte at a cathodic current density of about 50 to 100 amperes per square foot while maintaining the electrolyte at a temperature in the range of approximately 27° C. to 45° C., and during the elec-

trolysis replenishing the electrolyte with chrome alum to maintain the chromium content within the range between 18-60 grams per liter and adding a water soluble reduced sulphur compound at a rate of approximately 0.00002 to 0.0002 mol per liter per hour to maintain a concentration of about  $12 \times 10^{-5}$  mols per liter.

REX R. LLOYD.

#### REFERENCES CITED

The following references are of record in the file of this patent:

#### UNITED STATES PATENTS

| 15 | Number  | Name          | Date           |
|----|---------|---------------|----------------|
|    | 526,114 | Placet et al. | Sept. 18, 1894 |

#### FOREIGN PATENTS

| 20 | Number | Country       | Date           |
|----|--------|---------------|----------------|
|    | 19,344 | Great Britain | Sept. 26, 1890 |
|    | 22,855 | Great Britain | Nov. 19, 1891  |
|    | 18,743 | Great Britain | Aug. 5, 1899   |

#### OTHER REFERENCES

25 Rogers et al., Transactions of the Electrochemical Society, vol. 64 (1933), pages 299-304.